

## UNITED STATES PATENT OFFICE

2,008,302

## PROCESS OF PRODUCING ALLOYS CONTAINING YTTRIUM METALS OF THE RARE EARTHS

James B. Grenagle, Baltimore, Md., assignor of one-half to William W. Varney, Baltimore, Md., and one-half to Universal Alloys, Incorporated, Baltimore, Md., a corporation of Maryland

No Drawing. Application September 18, 1929,  
Serial No. 393,582

5 Claims. (Cl. 75—45)

My invention relates to improvements in the manufacture of steels and alloys, and while of general application to steel manufacture, it applies more particularly to the manufacture of 5 so-called alloy, or self-hardening steels, in which there is incorporated with the steel one or more metals of the yttrium group of the rare earths to produce steels or alloys suitable for tools and other articles requiring metals having special 10 hardness, toughness, tensile strength, etc. The object of my invention is to produce steels or alloys having better physical characteristics and also render such steels or alloys more uniform and free from defects.

According to my invention, I incorporate with the metal (scrap) a certain percentage of the oxalates of the yttrium group of the rare earths alone or in combination with other metals when operating by the crucible method, depending upon 20 the nature of the steel or alloy desired. The incorporation of the oxalates of the yttrium group of the rare earths improves the resulting steel or alloy in any case, and my invention in its broadest aspect comprehends the alloying of the yttrium 25 group of the rare earths in the manufacture of steel or alloys in general.

As a concrete example which gives satisfaction, an hydroxide of the earths is dissolved in an excess of oxalic acid and nearly neutralized with 30 ammonia; crystals form from the solution, and these crystals are washed, dried, powdered, etc., which gives me the oxalates I used.

According to my invention, I form a molten bath of low phosphorous pig iron of an approximate analysis, which I have found satisfactory, of carbon 2.50%, silicon 1 to 2%, manganese 1%, phosphorus .10%, and sulphur .05%. To this is added from 50 to 75% of steel scrap and brought 35 to a thoroughly molten condition. To this bath is added metallic concentrates of yttrium, or of the yttrium metals, alone or in combination with other metals, among which I might mention nickel, chromium, etc., depending upon the nature 40 of the steel or alloy desired. The incorporation of the metallic concentrates of the yttrium metals of the rare earths improves the resulting steel or alloy in any case, and my invention in its broadest aspect comprehends the alloying of the yttrium metals of the rare earths in the manufacture 45 of steel or alloys in general.

My invention relates more particularly to the so-called alloy steels or self-hardening steels, where the production of a superior high speed metal suitable for tools for lathes, shapers, drills, dies, etc., can be operated at a temperature of 50

2000° F.; for example, when used as a lathe tool it would stand a speeding up of the lathe to a heating point of the tool to 2000° F., retaining its cutting edge at that temperature.

The toughening and hardening properties given to the steel by the yttrium metals of the rare earths, are increased as compared with those given by vanadium, tungsten, chromium, molybdenum, cobalt, etc., supposedly on account of the lower specific gravity of the yttrium metals of the rare earths, as compared, for instance, with molybdenum or tungsten.

A given weight of the yttrium metals of the rare earths having a greater volume, will exert a greater influence. The oxides of molybdenum and tungsten, especially the former, are more volatile than those of the yttrium metal of the rare earths. In consequence of this, the effect of the yttrium metals of the rare earths is more permanent when the metal is heated.

Another advantage possessed by the yttrium metals of the rare earths is its resistance to the action of gases, such as, hydrogen. The yttrium metals of the rare earths also combine with any nitrogen or oxygen which may be present, thus purifying the metal bath and rendering the resultant metal more uniform.

The yttrium metals of the rare earths as metallic concentrates or metalloids, singly or in combination, may be added directly to the steel bath, or a ferro alloy containing the yttrium metals of the rare earths may be added to the steel bath, and after thoroughly liquefying, covering said bath with a suitable slag producing body to prevent vaporization of the metals; for example, an acid producing slag body from sands of substantially the following analysis: 45.70%  $Al_2O_3$ , 48.52%  $SiO_2$ , 3.08%  $Fe_2O_3$ , and 1.36%  $MgO$ , makes an excellent producing body.

The hot metal is cast in permanent molds, 40 made with iron flasks lined with a highly refractory oxide, or hydrate, insuring a clean, carbon-free metal. For example,  $Zr(OH_2)$  mixed with molasses water and formed under pressure in the mould, dried and calcined at a temperature of 45 2000° F., gives satisfactory results.

Another method is to reduce by means of carbon, using 4 or 5% of charcoal as a reducing agent, the yttrium metals of the rare earths directly from the ores, fergusonite, samarskite, 50 gadolinite, euxenite, etc.

I have discovered that the yttrium metals of the rare earths are particularly adapted to render the iron or steel alloys non-magnetic, presumably owing to the supposed fact that the iron in its 55

gaseous form is selectively occluded by certain of its elements in the yttrium metals of the rare earths group. I have discovered that as high as 90% of iron may be incorporated and the alloy will still be substantially non-magnetic.

I have also discovered that the non-magnetic quality of the alloys bears a distinct relation to its non-corrosive qualities, and this property in a large measure depends upon the supposed selective occlusion of other metals involved; as for example, yttrium is selective of iron and up to its saturation point renders the alloy free from attack on the iron occluded by it from its dissolving or oxidizing agent.

In high speed steel as now manufactured, the tungsten averages from 12% to 20%. According to my invention, if it is desired to replace the tungsten entirely with the yttrium metal of the rare earths, a less percentage of these, singly or in combination, may be used than the percentage of tungsten. In case all of the tungsten is not eliminated and it is desired to retain a certain percentage of the tungsten while having present the yttrium metals of the rare earths in less quantity than when they are used without the tungsten, the proper percentages may be determined readily by calculation. For example, about 3 to 6% of the yttrium metal of the rare earths may be used with a 6 to 10% of the tungsten.

The desired members of the yttrium metal of the rare earths may be introduced into the steel or alloy by introducing the concentrates and a suitable reducing agent, such as charcoal, or other suitable reducing agent.

Another method is to introduce them in the form of oxides, or the ferro alloy, just as is done in my U. S. Letters Patent No. 1,248,648, or my Letters Patent No. 1,385,072.

Still another method which may be used when it is desirable to incorporate other metals, such as hereinbefore referred to, is to combine the concentrates of the yttrium metals of the rare earths with the concentrates of these other metals and then throw the whole mixture into the steel bath; for example, the concentrates tungsten, molybdenum, chromium, etc., keeping the resulting metal in a freely fluid condition until free of sonims.

In the manufacture of ferrotungsten and ferrochrome, or other ferro additive alloys of this nature, the yttrium metal of the rare earths concentrated may be mixed with the concentrates of tungsten, molybdenum, chromium, etc., and incorporated with the iron to produce a ferrotungsten, ferrochrome, ferromolybdenum containing a certain percentage of the yttrium metal of the rare earths. This product can be distributed as a substitute for the present ferro alloys which are added to the bath in the production of these steels.

It will be understood that these are merely illustrations and that my invention is not limited to any particular proportions of the metals, but comprises in its scope the use of the yttrium metals of the rare earths alone in steel, or combined with other alloying metals. In this specification and claims, I describe my process and product to cover the yttrium metals of the rare earths in alloy form.

In this specification and claims, when I use the term, "yttrium metals of the rare earths", I mean, broadly, the yttrium metals of the rare earths group, one sample of which gives the following analysis; but I do not limit myself to the same, as all samples differ in analysis: Yttrium,

50%, dysprosium, 8%, holmium, 4%, erbium, 6%, thulium, 1%, ytterbium, 12%, lutecium 1%, terbium 8%, and contains probably unknown elements, and which I discovered as valuable to the alloys when introduced by means of the addition of the group as a whole.

The yttrium group taken as a whole forms an excellent deoxidizer for steel or cast iron. The advantage of using the yttrium group of metals for this purpose lies in the fact that it is cheaper to produce and has a much higher melting point, and less tendency to ignite and burn while being added to the ladle.

In reducing these yttrium earth concentrates or metals, I employ an electric furnace lined with a neutral lining made of rare earths oxide, preferably  $ZrO_2$ , and I employ 50 v. 1200 amperes until fusion takes place, and finally reduce current to 40 to 45 v. 600 amperes.

The concentrates I have used as set forth herein I obtained as follows—the process being the subject matter of a pending U. S. patent application Serial No. 387,268, issued into Patent No. 1,887,264, on November 8, 1932—the ores used being the yttrium group of the rare earths group: I break this into sizes suitable for my operating apparatus, preferably crushed and ground, but large size may be used. The apparatus used is a simple iron tank into which the ore is thrown mixed with sodium bisulphate, in the proportion of 1 lb. of the ore and 4 lbs. of sodium bisulphate. Two electrodes composed of sash-weight metal, a very hard iron of poor quality, containing perhaps silica and other impurities, are introduced into the mass content of the tank near the opposite sides thereof. Electric terminals are attached to these electrodes and a direct current is permitted to flow between the terminals; in the case illustrated, the diameter of the container being 40 inches and the electrodes being about 6 inches from the container on either side.

A current of 250 volts at 400 amperes was permitted to flow between the terminals for such a length of time as was necessary to reduce the mass to a fluid containing a precipitate, the period ranging from 3 to 7 hours, the time depending upon surrounding conditions, the current being run sufficiently long to entirely disintegrate the mass. The current used was a 3-phase current of 250 volts on the primary, 400 amperes passing through the reactance, the secondary showing about 120 volts at 800 amperes.

This latter current was what was used with a variable reactance for control, and was varied from 800 amperes to 250 amperes, as found convenient. The current was reduced to prevent excessive boiling, which was the principal controlling element, other than operating as fast as the boiling would permit. After precipitation, the liquid was siphoned off and the layers of precipitate were scraped off and the ore separated, the top layers containing probably yttrium co-mingled with various other lighter elements; the mother liquor also contained yttrium from which I obtained it by fractional crystallization, below which was chromium co-mingled with various elements of about its specific gravity, or forming imperfect precipitation. Below that came the heavier metals, gold, platinum and other rare elements in more or less impurity.

Having thus described my invention, what I claim and desire to secure by Letters Patent is:

1. The process of producing an alloy containing yttrium metals of the rare earths, consisting of introducing into a molten bath containing iron, 75

oxalates of the yttrium metals of the rare earths, bringing the entire mixture by fusion to liquefaction and while so doing protecting the said mass with a slag formed by a slag producing substance 5 introduced into said mass, then withdrawing said liquefied mixture from under said slag.

2. The process of producing an alloy containing the members of the yttrium metals of the rare earths consisting of reducing the yttrium 10 metals of the rare earths from their oxalates, said oxalates consisting substantially of the relative proportion of metals of yttrium 50%, dysprosium 8%, holmium 4%, erbium 6%, thulium 1%, ytterbium 12%, lutecium 1% and terbium 8%, by introducing the same into a bath of iron having as a 15 constituent carbon, then bringing the entire mass by fusion to liquefaction and while so doing protecting said mass by the slag formed by a slag producing substance introduced into said bath 20 whereby a hard pyro-alloy of iron and the yttrium metals of the rare earths is formed, then withdrawing from under said slag said molten alloy thus produced and formed.

3. The process of producing an alloy containing the members of the yttrium metals of the rare earths, consisting of reducing their oxalates in the presence of carbon by heat forming a molten bath thereof, protecting said bath with a slag 25 definitely formed for protective purposes, and 30 while so protected under said slag keeping the

mass in a freely molten fluid condition for an appreciable time to free the same from sonims, then diluting the said molten mass with another molten mass containing iron and maintaining the joint molten masses mixed at a temperature to maintain the same freely fluid for a sufficient time to thoroughly mix while in such molten condition, then withdrawing said molten mixture from under said slag into a refractory lined container.

4. The process of forming an alloy of iron consisting of melting iron into a molten bath and while in said molten condition adding carbon, and then adding thereto oxalates of the yttrium 10 metals of the rare earths by pouring the same on 15 the surface of said bath, thus permitting the same to permeate said bath to become reduced therein, whereby an alloy is formed having the property of a hard pyro-alloy.

5. The process of forming an alloy of iron consisting of forming a fused bath of iron having a carbon content, then adding thereto oxalates of 20 yttrium metals of the rare earths in excess of the amount required for reduction purposes whereby the excess may combine with the iron, 25 by pouring the same on the surface of said bath, thus permitting the same to permeate said bath to become reduced therein whereby an alloy is formed having the property of a hard pyro-alloy.

JAMES B. GRENALE. 30